

March 30, 1937.

A. W. THOMPSON

2,075,410

IMPREGNATED DIELECTRIC MATERIALS AND IMPREGNATING COMPOSITIONS

Filed Dec. 4, 1935



INVENTOR:  
Archibald Walter Thompson,  
By Stebbins, Blenko & Pannell,  
Atty.

## UNITED STATES PATENT OFFICE

2,075,410

IMPREGNATED DIELECTRIC MATERIALS  
AND IMPREGNATING COMPOSITIONS

Archibald Walter Thompson, Bromley, England

Application December 4, 1935, Serial No. 52,885  
In Great Britain December 13, 1934

13 Claims. (Cl. 154—2.6)

This invention consists in improvements in or relating to impregnated dielectric materials suitable for cable wrappings or interleaving sheets for condensers or for like purposes. An object 5 of the invention is to produce an insulating material having high resistance to oxidation and good dielectric properties.

It is customary to impregnate paper or like wrappings for electric cables with oil but difficulties arise in practice because the oil is apt to drain away from the paper or the like. Mixtures of oil and resin having a high viscosity are commonly employed to impregnate paper or like wrappings with a view to obviating draining but 15 such mixtures are susceptible to oxidation and it is found difficult to obtain sufficiently good dielectric properties.

It has now been discovered that hydrocarbons of very high viscosity (e. g. 2000 to 3000 seconds Redwood at 200° F.) may be obtained by polymerizing suitable petroleum fractions in the presence of certain metallic chlorides, e. g. aluminium chloride.

According to this invention an impregnated dielectric material comprises paper or like absorbent fibrous material impregnated with a mixture of a highly viscous hydrocarbon, having a viscosity value between the limits 2500 and 3000 seconds Redwood at 200° F., with a less viscous mineral oil having a viscosity value less than 200 seconds Redwood at 200° F. The mixture is a homogeneous mixture of the oils and should have a viscosity value of between 1500 and 3000 seconds Redwood at 140° F. Preferably the high viscosity hydrocarbon is refined, before mixing, by any suitable refining process, for example by treatment with selective solvents (e. g. the Duosol process) or with liquid sulphur dioxide or by acid treatment or alkali treatment or by bleaching 30 with earths or by high vacuum distillation.

In order to reduce the likelihood of gassing or "cheese" formation in the dielectric material under electric stress (which commonly results when a saturated paraffinic or olefinic oil is employed) it is a further feature of the invention to use, as the mineral oil (which should preferably have a viscosity value between 50 and 200 seconds Redwood at 200° F.), a pure, highly refined naphthenic oil e. g. the Sun Oil Company's XX oil. Preferably the mixture comprises 30% of said highly viscous hydrocarbon.

The invention includes an electric cable wrapped with paper or like absorbent fibrous material (e. g. jute) impregnated with the mixture described. Preferably the impregnation is

carried out during or after the wrapping steps.

In one specific example of the invention which will now be described, a high viscosity hydrocarbon was prepared by polymerizing the heavy ends from a petrol produced by cracking crude oil, in the presence of anhydrous aluminium chloride, the polymerization being carried out in the vapour phase, and to the full extent so as to give the maximum viscosity. The high viscosity product so obtained was mixed with highly refined naphthenic oil in the proportions of one part of the product to two parts of the oil. This mixture has a viscosity of 2,500 seconds Redwood at 60° C. so being in accordance with normal European practice, and was employed to impregnate a paper-wrapped electric cable.

Any suitable petroleum fraction (e. g. any fraction between petrol and fuel oil) may be polymerized to give the high viscosity product and the polymerization may be carried out in either the liquid or vapour phase.

It is found that a cable wrapped with paper impregnated with the mixture described has a particularly high dielectric resistance, and resistance to oxidation as well as low power factor losses and that the cable may be operated at temperatures up to 20 to 30° C. higher than is the usual practice without causing thermal instability and subsequent breakdown. The size of the cable and consequently the cost may therefore be decreased without sacrifice of safety.

The drawing is a diagrammatic representation of an electric cable provided with an insulating covering formed from a strip of absorbent fibrous material wrapped around the electric conductor and impregnated either before or during the wrapping operation with the hydrocarbon mixture hereinbefore described. The cable may be provided with the usual protective sheath of any suitable material.

The invention includes the use, as an impregnating medium for dielectric materials, of a mixture of a hydrocarbon of high viscosity and a comparatively low viscosity mineral oil.

I claim:—

1. An impregnated dielectric material comprising an absorbent fibrous material impregnated with a mixture of a highly viscous hydrocarbon, having a viscosity value between 2500 and 3000 seconds Redwood at 200° F., with a less viscous mineral oil having a viscosity value of less than 200 seconds Redwood at 200° F.

2. An impregnated dielectric material comprising an absorbent fibrous material impregnated with a mixture of a highly viscous hydrocarbon,

having a viscosity value between 2500 and 3000 seconds Redwood at 200° F., with a less viscous mineral oil having a viscosity value between 50 and 200 seconds Redwood at 200° F., which mixture has a viscosity value between 1500 and 3000 seconds Redwood at 140° F.

3. An impregnated dielectric material comprising an absorbent fibrous material impregnated with a mixture of a highly viscous refined hydrocarbon, having a viscosity value between 2500 and 3000 seconds Redwood at 200° F., with a less viscous mineral oil having a viscosity value of less than 200 seconds Redwood at 200° F.

4. An impregnated dielectric material comprising an absorbent fibrous material impregnated with a mixture of a highly viscous hydrocarbon, having a viscosity value between 2500 and 3000 seconds Redwood at 200° F., with a highly refined naphthenic oil having a viscosity value of less than 200 seconds Redwood at 200° F.

5. An impregnated dielectric material comprising an absorbent fibrous material impregnated with a mixture of a highly viscous hydrocarbon, having a viscosity value between 2500 and 3000 seconds Redwood at 200° F., with a less viscous mineral oil having a viscosity value between 50 and 200 seconds Redwood at 200° F., which mixture has a viscosity value between 1500 and 3000 seconds Redwood at 140° F., said mixture containing about 30% of said highly viscous hydrocarbon.

6. An impregnated dielectric material comprising paper impregnated with a mixture of a highly viscous hydrocarbon, having a viscosity value between 2500 and 3000 seconds Redwood at 200° F., with a less viscous mineral oil having a viscosity value of less than 200 seconds Redwood at 200° F.

7. An impregnated dielectric material comprising paper impregnated with a mixture of a highly viscous refined hydrocarbon, having a viscosity value between 2500 and 3000 seconds Redwood at 200° F., with a highly refined naphthenic oil having a viscosity value between 50 and 200 seconds Redwood at 200° F., which mixture has a viscosity value between 1500 and 3000 seconds Redwood at 140° F.

8. An impregnated dielectric material comprising paper impregnated with a mixture of a highly viscous refined hydrocarbon, having a viscosity

value between 2500 and 3000 seconds Redwood at 200° F., with a highly refined naphthenic oil having a viscosity value between 50 and 200 seconds Redwood at 200° F., which mixture has a viscosity value between 1500 and 3000 seconds Redwood at 140° F., said mixture containing about 30% of said highly viscous refined hydrocarbon.

9. An impregnated dielectric material for an electric conductor comprising a strip of absorbent fibrous material wrapped around said conductor and impregnated with a mixture of a highly viscous refined hydrocarbon, having a viscosity value between 2500 and 3000 seconds Redwood at 200° F., with a highly refined naphthenic oil having a viscosity value between 50 and 200 seconds Redwood at 200° F., which mixture has a viscosity value between 1500 and 3000 seconds Redwood at 140° F., said mixture containing about 30% of said highly viscous refined hydrocarbon.

10. An impregnating medium for dielectric materials comprising a mixture of a highly viscous hydrocarbon, having a viscosity value between 2500 and 3000 seconds Redwood at 200° F., with a less viscous mineral oil having a viscosity value of less than 200 seconds Redwood at 200° F.

11. An impregnating medium for dielectric materials comprising a mixture of a highly viscous hydrocarbon, having a viscosity value between 2500 and 3000 seconds Redwood at 200° F., with a highly refined naphthenic oil, having a viscosity value of less than 200 seconds Redwood at 200° F.

12. An impregnating medium for dielectric materials comprising a mixture of a highly viscous hydrocarbon, having a viscosity value between 2500 and 3000 seconds Redwood at 200° F., with a highly refined naphthenic oil, having a viscosity value between 50 and 200 seconds Redwood at 200° F., said mixture containing about 30% of said highly viscous hydrocarbon and having a viscosity value between 1500 and 3000 seconds Redwood at 140° F.

13. An impregnated dielectric material comprising an absorbent fibrous material impregnated with a mixture of a highly viscous hydrocarbon, having a viscosity value between 1500 and 3000 seconds Redwood at 200° F., with a less viscous mineral oil having a viscosity value of less than 200 seconds Redwood at 200° F.

ARCHIBALD WALTER THOMPSON.